

Mar. 20, 1923.

1,448,928

R. LUCKENBACH

METHOD OF CONCENTRATING ORE

Filed Apr. 5, 1918



Witnesses

*A. Weston*  
*C. Goline*

Inventor  
Royal Luckenbach  
By *Alfred Gaynor*  
Attorney

## UNITED STATES PATENT OFFICE.

ROYER LUCKENBACH, OF BROOKLYN, NEW YORK, ASSIGNOR TO LUCKENBACH PROCESSES, INC., OF SAN FRANCISCO, CALIFORNIA, A CORPORATION OF NEVADA.

## METHOD OF CONCENTRATING ORES.

Application filed April 5, 1918. Serial No. 226,634.

To all whom it may concern:

Be it known that I, ROYER LUCKENBACH, a citizen of the United States, residing in the borough of Brooklyn, county of Kings, 5 city and State of New York, have invented a certain new and useful Method of Concentrating Ores, of which the following is a specification.

This invention relates to the concentration 10 of ore in which the valuable mineral constituents are separated from the valueless earthy or rocky content or gangue with which they are naturally associated. In the practice of the invention advantage is taken 15 of the known preferential affinity of certain substances for certain minerals which will attract, or be attracted by, such substances while at the same time the silicious gangue will not be so attracted but will be repelled. 20 The invention is particularly directed to what may be termed the contact method of ore concentration in which the ore, in finely divided state, is mixed with water to form a pulp which is then brought into contact 25 with a surface to which the mineral content of the ore will adhere.

The invention comprises the employment 30 of a selective agent having a great affinity for certain minerals and which will not attract or be attracted by gangue. The invention also comprises the method or process 35 of utilizing such a selective agent.

The objects and advantages of the invention will be appreciated from a reading of 35 the following specification and claims.

The invention is applicable to the treatment 40 of metals in the free or virgin state as well as certain chemical combinations thereof. By the process of the invention metallic minerals and their sulphides may be separated from the earthy gangue with which they are associated, and likewise certain non-metallic minerals, such for example as sulphur and graphite, may be concentrated.

45 In addition to separating the valuable content of ores having a flinty or rocky gangue, the process may be carried out in connection with free metals found in placer or surface mining.

50 The invention may be carried out with all ores and their chemical compounds which are subject to concentration by the oil flotation methods at present in use, as well as with other mineral substances which will

not be acted on by the materials employed 55 in the oil flotation processes.

For the purposes of carrying out the invention the selective material or agent comprises an unctuous material of animal, vegetable or mineral origin, a resinous material 60 of which caoutchouc, copal, rosin, shellac, asphaltum, Burgundy pitch and North Carolina pitch are examples, or a combination of such unctuous and resinous materials.

The resin is rendered suitable for use in 65 the invention by dissolving it in a suitable solvent, having water repellent characteristics. The oily or greasy substance when of a heavy, thick nature is preferably thinned to a proper consistency by the addition of a thin oil.

Specifically the preferred selective agent comprises petroleum grease and rubber. The rubber, preferably Para rubber, is prepared by dissolving it in a hydrocarbon 75 solvent such as near-turpentine or other suitable solvent. Near-turpentine is a petroleum distillate from which the fat or grease has been removed. It is a clear, limpid liquid having the appearance of gasoline, benzene, 80 or naphtha, and the odor of kerosene and is employed because of its cheapness, but many other rubber solvents may be employed, such, for example, as carbon disulphide. The petroleum grease which is naturally a 85 thick, heavy substance is thinned by the rubber solvent, or any other suitable material, to such an extent that it is capable of use in the process.

Petroleum grease and rubber when thus 90 treated and combined produce a mixture having a consistency of approximately that of syrup. They may be combined in substantially equal proportions which will produce this liquor of the desired syrupy nature. The proportions of grease and rubber may vary considerably as depends upon the quality or kind of ore acted upon, and for various other reasons.

In the accompanying drawings, in which 100 like parts in all of the figures are designated by similar characters of reference, are illustrated several means by which the process may be carried out, and in which—

Fig. 1 is a diagrammatic view of a belt 105 vanner arrangement.

Fig. 2 is a modification showing a cylinder for carrying the pulp.

Fig. 3 shows the use of a revolving table, and

Fig. 4 illustrates an inclined chute.

The mixture of petroleum grease and rubber is placed, in the form of a thin coating, upon the surface of a continuously moving belt 1, for example. The ore pulp composed of ore and water is directed to the coated surface from a hopper 2 whereupon the mineral constituents of the ore will adhere to the coating and the water and gangue will not adhere to the surface but will be discharged from the belt when the latter changes its direction of travel into a trough of launder 3. The coating will adhere to the belt and the mineral matter will be retained in contact with the coating against dislodgment by centrifugal force or by agitation. The coating with the adhering mineral will be removed from the belt in any desired manner, as by means of a scraper 4 and directed into a receptacle 5. The surface of the belt is re-coated automatically as from a reservoir 6 or otherwise and the operations are repeated whereby the process is continuous.

The mineral and the selective agent, after removal from the belt, are separated in any suitable manner. The separation may take place in a hot water bath in which the composition will be melted, the resinous and oily materials will float on the surface of the water and the mineral matter will sink and form a perfectly clean concentrate. The selective may be recovered from the water of the bath and re-used.

Instead of employing a hot water bath for separating the mineral from the selective agent the separation may be effected in a press or centrifugal machine.

If the recovery of the selective agent is not a consideration, it,—the agent,—may be removed from the concentrates by a suitable solvent of the agent or by burning.

Instead of a moving belt the coating may be applied to a rotating or rocking table 7, to the surface of a cylinder 8, or to an inclined chute 9 along which the pulp may be caused to flow.

When the rotating table 7 is employed the gangue and water may be expelled by centrifugal force. The surface of the table may be scraped and dressed as in the method shown in Fig. 1, or the table may be coated and scraped by hand.

In the method illustrated in Fig. 4 the chute 9 is coated by hand, the water and gangue will travel along the surface by gravity, the values will adhere to the surface and the chute may be scraped at the end of the run.

The contact method of ore concentration employing the selective agent herein disclosed possesses many advantages over the oil flotation methods now in use. It per-

mits of operation with ore much coarser than is possible in flotation processes. In the latter case the ore must be ground to 80 or 100 mesh in order that the metallic particles will be light enough to be borne to the surface in the froth of flotation. In the process of this invention it is not necessary to float the mineral and the ore need not be ground to a degree of fineness exceeding 30 mesh. This will reduce the expense of grinding and the present process will permit of a much greater recovery of mineral in the same length of time than is possible by the flotation methods.

The contact method is also more economical than the flotation system for the reason that it requires less power, is automatic, and continuous.

In the flotation process the oil may be used but once as it cannot be recovered, whereas in the process of the present invention the selective agent may be recovered and re-used.

It is to be understood that the selective agent comprising petroleum grease and liquid rubber above described is the preferred selective agent but it is not the intention to limit the invention to the use of such an agent.

Liquid rubber alone may be employed as the mineral selective agent and will give excellent results. Petroleum grease alone may be used. When so employed the grease must be cut to a syrupy consistency, preferably by the use of a thin liquid hydro-carbon solvent. The addition of liquid rubber to petroleum grease increases the mineral selective qualities of the latter in proportion to the amount of rubber used.

Any of the suitable resins or oils alone may be used as the mineral selective agent for the purposes of this invention, it being understood, that the resins will be previously dissolved in a suitable solvent, for use in the form of a coating for the belt, or other surface of the apparatus, to which the ore pulp is to be directed. Certain of the oils which may be used as a mineral selective agent must be modified to produce a coating which will be of a slippery, slimy, or "slick" character rather than of a gluey or tacky nature. For example, if asphaltum were to be used it would be so tacky or gluey that it would retain both the mineral and the gangue upon the belt instead of separating the mineral from the gangue, but when asphaltum is combined with a fatty acid it loses its character of tackiness and becomes of a sufficiently smooth or "slick" character to serve as a gangue repellent while retaining its mineral selective qualities.

For the purpose of more efficient action as a mineral selector therefore, it is preferable to combine a resinous and an oleaginous substance, as the combination of the two

substances tends to increase the selectiveness, for mineral, of both. The addition of the resin, especially rubber, causes the oily substance to adhere to the belt and tends to remove the tendency of the oils (which tendency is greater in some oils than in others) to float off the belt, or other contact surface, in the water of the ore pulp, or to scour off by the gangue. Rubber also provides a protective, water-proof coating for the belt and protects it from injury.

The liquid rubber imparts to the oil or grease an added quality of cohesion and of resistance to water, thus preventing the oil from dissipating.

Having thus described my invention, what I claim is:—

1. The method of concentrating ore, which comprises mixing the ore with water to form a pulp, directing the pulp to a surface comprising petroleum grease and rubber to which the mineral content will ad-

here, and separating the mineral from the material.

2. The method of concentrating ore, which comprises mixing the ore with water to form a pulp, directing the pulp to a surface comprising petroleum grease and liquid rubber to which the mineral content will adhere, and separating the mineral from the material.

3. The method of concentrating ore, which comprises mixing the ore with water to form a pulp, directing the pulp to a surface comprising petroleum grease and rubber dissolved in a hydro-carbon to which the mineral content will adhere, and separating the mineral from the material.

This specification signed and witnessed this thirtieth day of March, 1918.

ROYER LUCKENBACH.

Witnesses:

A. E. RENTON,  
M. I. WARD.